

## UNITED STATES PATENT OFFICE.

ERNST OESER, OF SCHÖNEBERG, NEAR BERLIN, GERMANY, ASSIGNOR  
TO GENTHINER CARTONPAPIER-FABRIK G. M. B. H., OF BERLIN,  
GERMANY.

## METHOD OF MANUFACTURING THIN BRONZE OR OTHER METAL PLATES.

SPECIFICATION forming part of Letters Patent No. 788,940, dated May 2, 1905.

Application filed November 14, 1903. Serial No. 181,216.

*To all whom it may concern:*

Be it known that I, ERNST OESER, manufacturer, a subject of the German Emperor, residing at No. 19-20 Bahnstrasse, in the city of 5 Schöneberg, near Berlin, in the Kingdom of Prussia, German Empire, have invented certain new and useful Improvements in Methods for the Manufacture of Thin Bronze or other Metal Plates, of which the following is 10 a full and exact specification.

This invention relates to an improved method for the manufacture of thin bronze or other metal plates.

For the purpose of manufacturing metal 15 stampings or printings on paper, leather, or the like it has been usual to use sheet metal and a suitable grounding and binding agent or adhesive; but the sheet metal has the disadvantage that with fine ornaments or with 20 very small letters the patterns do not come out sharp enough and that frequently the object to be treated is impaired by the use of grounding and binding agents. It has also been attempted to manufacture metal stampings and printings by powdering the part to 25 be treated with bronze-powder and then pressing the die upon it. By this method, on the one hand, incompletely-covered stampings are produced, and, on the other hand, the stamping or pattern has a dead appearance, the so-called "bronze" stampings never filling the place of those produced by the use of the sheet metal.

In order to quickly and conveniently produce polished metal stampings by means of bronze or metal powder, the said metal powder is combined with a thin layer of color in any suitable manner and laid on the part to be printed or patterned similarly to a thin 35 plate of metal without using any grounding or adhesive agent. The manufacture of such thin bronze plates is the object of the present invention, and according thereto the color mass is laid thinly on a glass plate, which 40 serves first as a support for the bronze-powder, and then said mass is scattered over with the bronze-powder through a suitable sifting device. When dry, the superfluous bronze-

powder is removed with a soft brush and the thin layer or plate taken off in the known 50 manner with a pallet-knife. The mass is composed in a similar manner to the known thin plates of color—that is to say, they consist of size, glycerin, a suitable powdered color—as, for instance, zinc-white, ocher, or 55 the like—water, and albumen. It not only acts as a support, but also as grounding and binding agent, and gives the bronze-powder the necessary polish on the stamping. It will be seen that variously-colored bronze-powders 60 can be used for the manufacture of said thin bronze plates, and, if necessary, it may be laid on the already-painted layer in such a manner that the color becomes iridescent in order to produce an iridescent effect in the metal 65 stampings or printings.

What I claim as my invention, and desire to secure by Letters Patent of the United States, is—

1. A method for the manufacture of thin 70 bronze plates for stampings and printings consisting in laying a liquid mass of size and glycerin on a smooth surface, scattering the bronze or other metal powder upon said layer, while still moist, and removing the layer and 75 metal coating when dry from said surface substantially as described.

2. A process for producing bronze-leaf, consisting in forming upon a smooth surface a layer of binding and cohesive material in a 80 moist state, sifting finely-divided bronze thereupon while the former is in a moist state, allowing the product to dry, and removing the same from said smooth surface in the form of a leaf or foil.

3. A process of producing metal leaves for stamping purposes, which consists in forming upon a smooth surface a liquid bottom layer of adhesive material, scattering metal powder on the bottom layer while still moist 90 to form a non-adhesive top layer thereon, and removing the product from the smooth surface when dry.

4. A process of producing metal leaves for stamping purposes, which consists in forming 95 upon a smooth surface a liquid bottom layer

of adhesive and coloring material, allowing the layer to partly dry, then scattering metal powder on the bottom layer to form a non-adhesive top layer thereon, allowing the product to completely dry, then removing the superfluous metal powder, and finally removing the product from the smooth surface.

The foregoing specification signed at Berlin this 3d day of November, 1903.

ERNST OESEER.

In presence of—  
HENRY HASPER,  
WOLDEMAR HAUPT.